

Sullivan, 3rd et al.

[45]

**June 7, 1977**

## [54] HIGH TEMPERATURE CORROSION INHIBITOR

|           |         |                        |            |
|-----------|---------|------------------------|------------|
| 3,127,447 | 3/1964  | Jaruzelski et al. .... | 252/148 X  |
| 3,696,048 | 10/1972 | Hausler et al. ....    | 252/390 X  |
| 3,779,935 | 12/1973 | McDougall et al. ....  | 252/8.55 X |

[75] Inventors: **Daniel S. Sullivan, 3rd, Houston, Tex.; Charles E. Strubelt, Tamare, Venezuela; Kenneth W. Becker, Houston, Tex.**

*Primary Examiner*—Herbert B. Guynn  
*Attorney, Agent, or Firm*—David A. Roth; C. Leon Kim

[73] Assignee: **Exxon Research and Engineering Company, Linden, N.J.**

[22] Filed: Dec. 3, 1975

[21] Appl. No.: **637,168**  
[52] U.S. Cl. ..... **252/392; 252/8.55 C;**  
..... **252/390**

[51] Int. Cl.<sup>2</sup> ..... C23F 11/04  
[58] Field of Search ..... 252/8.55 C, 8.55 E,

[58] Yield of Search ..... 252/3,333 C, 3,333 E,  
252/148, 390, 392

[56] References Cited

UNITED STATES PATENTS

|           |         |                         |           |
|-----------|---------|-------------------------|-----------|
| 2,037,762 | 4/1936  | Cole .....              | 252/148   |
| 2,814,593 | 11/1957 | Beiswanger et al. ..... | 252/8.55  |
| 3,113,113 | 12/1963 | Marsh et al. .....      | 252/148 X |

[57] ABSTRACT

Metal corrosion inhibiting compositions of outstanding utility are prepared by utilizing a selective and critical multicomponent formulation comprising in combination functionally operative proportions of

a specific quaternized cyclic nitrogen base  
a specific acetylenic alcohol  
a surface active agent  
a formic acid derivative.

The above formulation can be substantially improved by adding certain functionally operative additional surfactants. The choice of these surfactants is unobvious and it has been found that only a few critically selective species are operable for the purposes of the invention.

**22 Claims, No Drawings**

**HIGH TEMPERATURE CORROSION INHIBITOR****CROSS REFERENCE TO RELATED APPLICATIONS**

This application is not related to any pending patent application or issued patent of these inventors.

**BACKGROUND OF THE INVENTION****1. Field of the Invention**

This invention relates to corrosion inhibitor compositions and is particularly concerned with multicomponent inhibitor formulations capable of protecting ferrous metals against attack by corrosive acids in high temperature environments.

**2. Description of the Prior Art**

The corrosion of oil field tubular goods and similar equipment by hydrochloric acid solutions and other corrosive materials used in well workover and stimulation operations is a longstanding problem in the petroleum industry. The use of inhibitors to combat such corrosion is conventional. The materials suggested in the past for use in such inhibitors include various acetylenic alcohols, fluorinated surfactants, quaternary derivatives of heterocyclic nitrogen bases and halomethylated aromatic compounds, formamides, and surface active agents, alone or in combination with other materials. U.S. Pat. No. 2,814,593, for instance, discloses compositions of this nature. Tests have shown that certain of these earlier compositions are reasonably effective for inhibiting the corrosion of ferrous metals in shallow wells where temperatures are relatively low and conditions are not severe. In deeper wells where temperatures of 300° F. or higher are apt to be encountered, it has been found that corrosion rates tend to be exceptionally high and that many of the compositions advocated for use in the past are inadequate. Efforts to develop improved inhibitors which will be effective under these more severe conditions have not heretofore been as promising as the compositions of the instant invention.

**SUMMARY OF THE INVENTION**

This invention comprehends a specific formulation of components for a corrosion inhibitor composition which is considerably more effective than inhibitors available in the past. In accordance with the invention, it has now been found that an inhibitor formulation which is surprisingly effective for the protection of ferrous metals against attack by corrosive acids at elevated temperatures can be prepared by blending at least four unique specially selected components which unexpectedly interact together to result in an outstanding corrosion inhibitor composition.

**DESCRIPTION OF THE PREFERRED EMBODIMENTS****A. The Quaternized Cyclic Nitrogen Base and Polystyrenes**

The quaternary compounds which have been found useful as one component for preparing the improved inhibitor composition of the invention are quaternary derivatives of quinoline and halomethylated polycyclic compounds selected from the group consisting of halomethylated polynuclear aromatics containing from 2 to 4 condensed aromatic rings per molecule, mixtures

of such halomethylated polynuclear aromatics, and halomethylated polystyrene.

Polynuclear aromatics which can be halomethylated and employed for purposes of the invention include 5 indane, indene, naphthalene, methyl naphthalene, anthracene, phenanthrene, acenaphthene, fluorene, xanthene, chrysene, pyrene and the like.

These compounds can be isolated and individually halomethylated if desired, but in most cases, it is preferred 10 to employ mixed polynuclear aromatics derived from crude oil, petroleum fractions or coal tar.

Alternatively, petroleum fractions or other oils containing polynuclear aromatic compounds can be subjected to halomethylation, followed by recovery of the 15 halomethylated product. Depending upon the particular oil selected, this latter procedure may result in the inclusion of some halomethylated single ring aromatic compounds, but the presence of such materials in reasonably small quantities is not ordinarily objectionable. 20 Oils suitable for halomethylation to produce the mixed halomethylated products include aromatic solvents boiling within the range of about 200° and about 750° F. and similar petroleum fractions.

The polystyrenes which may be halomethylated and 25 used in preparing the inhibitor compositions of the invention will normally be low molecular weight polymers. Polystyrenes having molecular weights in the range between about 100 and about 5000 are normally preferred and those with molecular weights between 30 about 100 and about 500 are particularly effective for purposes of the invention.

The polynuclear aromatic compounds and polystyrenes which are used in the preparation of the quaternary compounds employed as a component of the inhibitor blends of the invention can be halomethylated by treating them with a hydrogen halide gas in the 35 presence of paraformaldehyde and anhydrous zinc chloride in a stirred reactor. The aromatic material, paraformaldehyde and zinc chloride are first charged to the reactor and then brought up to the reaction temperature of about 130° to about 150° C. while providing agitation. The hydrogen halide gas is then introduced into the reaction mixture at a rate which will 40 permit control of the temperature. Upon completion of the reaction, the reaction mixture can be cooled, diluted with water, and then extracted with ether or a similar solvent to recover the halomethylated product. The solvent can then be removed by distillation. The 45 product can then be washed to further purify it and then dried for use in preparing the quaternary compound. Other conventional halomethylation procedures can also be employed.

The quaternarization reaction of the halomethylated 50 polycyclic material with quinoline or a similar heterocyclic nitrogen base is normally carried out in isopropanol, formamide or a similar solvent at a temperature between about 200° and about 250° F. After the reaction has been completed, the product can be cooled 55 and diluted with additional solvent to produce a solution in a concentration suitable for use in preparing the inhibitor compositions of the invention. Concentrations on the order of about 40 to about 75% by weight are normally preferred. It will be understood, of course, 60 that preparation of the quaternary derivatives employed is not restricted to this particular process and that other conventional quaternarization processes 65 may be used.

## B. Specific Acetylenic Alcohol

The acetylenic alcohols employed in the improved inhibitor compositions are aliphatic alcohols which contain from 3 to about 10 carbon atoms per molecule and have the general formula:



where  $R_1$  is selected from the group consisting of the hydrogen atom and the methyl group and  $R_2$  is selected from the group consisting of the hydrogen atom and alkyl groups containing up to about 7 carbon atoms. Suitable acetylenic alcohols of this type include propargyl alcohol, 1-butyn-3-ol, 3-methyl-1-butyn-3-ol, 1-pentyn-3-ol, 3-methyl-1-pentyn-3-ol, 1-hexyn-3-ol, 3-methyl-1-hexyn-3-ol, 1-octyn-3-ol, hexyne-1-ol-3, 20 hexyne-1-methyl-3-ol-3,4-ethyl-1-octyn-3-ol and the like. The use of mixtures containing two or more such alcohols is generally preferred. Alcohols of this type and such mixtures are available commercially.

## C. The Surface Active Agent

A variety of different surface active agents can be employed in the compositions of the invention. The surface active agent serves as a dispersing material and wetting agent and aids in reducing the amount of pitting which takes place. The preferred surface active agent is a nonionic ethylene oxide adduct of a primary amine having the structural formula:



where  $R$  is  $C_5$  to  $C_{50}$  alkyl group, preferably an aliphatic or substituted aliphatic chain containing from about 12 to about 18 carbon atoms and  $x$  and  $y$  are numbers ranging from 1 to 20, preferably between 1 and about 4. The preferred compounds are those which contain aliphatic groups derived from naturally occurring materials such as tallow, coconut oil and soybean oil and which contain from 1 to 3 ethylene oxide groups in each of the ethylene oxide chains attached to the nitrogen atom. Compounds which are particularly effective for purposes of the invention include those having the following structural formulas:



As indicated earlier, the invention is not restricted to the particular surface active agents described above and can instead be practiced with a variety of other surfactants. Representative materials which can be used include aliphatic primary amines containing from about 12 to 18 carbon atoms per molecule, secondary amines containing a methyl group and a  $C_{12}$  to  $C_{18}$  alkyl group, tertiary amines containing two methyl groups and a  $C_{12}$  to  $C_{18}$  alkyl group,  $C_{12}$  to  $C_{18}$  alkyltrimethylammonium chlorides, polyethoxylated ethers of aliphatic alcohols, polyethoxylated esters of fatty acids, 65 polyethylene oxide adducts of alkyl phenols, tall oils, and the like. A variety of such surface active agents which will be suitable for purposes of the invention are

25

30

40

45

50

60

available commercially and will be familiar to those skilled in the art.

## C(1). The Supplemental Surface Active Agent

Regardless of the particular surface active agent utilized as described above, an additional important improvement facet of this invention resides in the use of a special supplemental surface active agent in the formulation.

10 The supplemental agent is a lauryl alcohol derivative of ethylene oxide with about 20 to 23 moles of ethylene oxide forming the polyether adduct of the alcohol.

A preferred supplemental agent is available commercially as BR1J-35 from Atlas Chemical Company.

15 It is used in quantities of from 6 to 14, preferably 8 to 12, and most preferably 9 to 11 weight percent based on the total weight of the active components of the four major component formulation of the invention.

This supplemental agent plays an important role in commercial formulations, since it prevents precipitation of the formulation under adverse field conditions.

Precipitation is undesirable since it causes cleaning problems for field equipment: tanks, tank trucks and the like.

## D. The Formic Acid Derivatives

The formic acid derivatives which are employed in preparing the improved corrosion inhibitor formulations are compounds having the formula:



35 where  $Z$  is chosen from the group consisting of an alkoxy group containing from about 1 to about 4 carbon atoms, an amino radical, or an alkyl-substituted amino group containing from 1 to about 4 carbon atoms. Specific examples of such compounds include methylformate, ethylformate, butylformate, formamide, dimethylformamide, diethylformamide, and the like. Compounds of this type are commercially available from a variety of different sources. The use of formamide is normally preferred.

## E. The Fluorinated Surfactant (Optional)

A typical fluorinated surfactant suitable for this invention is marketed commercially as FC-134, however many cationic fluorinated surfactants are suitable. Perfluoroalkylimidazolines can also be used.

## F. Preparation Details

The improved inhibitor compositions of the invention are prepared by blending the constituents in the disclosed concentrations in a vat or other vessel provided with a suitable agitator. Typical amounts of the various components are shown below:

| Constituent                                                         | Concentration                                            |
|---------------------------------------------------------------------|----------------------------------------------------------|
| Quaternary derivative of quinoline and polycyclic aromatic compound | About 25 to about 60, preferably 30 to 50 weight percent |
| Acetylenic alcohol                                                  | About 5 to about 30, preferably 8 to 15 weight percent   |
| Surface active agent                                                | About 0.01 to about 15, preferably 1 to 5 weight percent |
| Formic acid derivative                                              | About 30 to about 75,                                    |

-continued

| Constituent            | Concentration                                         |
|------------------------|-------------------------------------------------------|
|                        | preferably 40 to 60 weight percent                    |
| Fluorinated surfactant | 0 to about 1.0, preferably 0.05 to 0.8 weight percent |

The inhibitor compositions of the invention formulated as described above can be used in any of a variety of applications requiring the protection of ferrous metals against attack by corrosive acids but are particularly useful for inhibiting the corrosion of oil well tubular goods and similar equipment by hydrochloric acid and other acid solutions used in workover and stimulation operations for high temperature oil and gas wells. The inhibitor compositions of the invention are normally incorporated in such acid solutions in concentrations ranging from about 0.1 to about 5% by weight. The concentration selected for a particular application will depend in part upon the particular acid solution then used, the susceptibility of the tubular good or other ferrous material to corrosion by the acid, and the environment in which the acid is to be employed. Concentrations between about 0.5 and about 3% by weight are generally preferred.

The invention is further illustrated by the following examples.

#### EXAMPLE 1

In the first of a series of laboratory experiments, a reactor was charged with 123 g. of crude quinoline and 140 g. of 1-(chloromethyl)naphthalene. The contents of the reactor were stirred and the vessel was then heated to a temperature of 125° C. Following this, a small portion of a total 176 g. quantity of isopropyl alcohol was added to the reactor and refluxing of the reaction mixture was started in order to maintain the reaction mixture at the 125° C. temperature. This was continued for a period of about 3 hours, the temperature remaining relatively constant at about 125° C.

At the end of this period the reaction product was slowly cooled to room temperature and the remainder of the 176 g. of isopropyl alcohol was blended into the product. The result was an isopropyl alcohol solution containing 60% by weight of N-(1-naphthylmethyl)-quinolinium chloride. This quaternary derivative of quinoline and a halomethylated polynuclear aromatic compound is a useful species of one constituent of the improved corrosion inhibitor compositions of the invention.

#### EXAMPLE 2

A quaternary derivative of quinoline and phenanthrene was prepared by first charging 267.3 g. of phenanthrene, 82.5 g. of paraformaldehyde, 195 mm of glacial acetic acid, 124 mm of 85% phosphoric acid and 321 g. of concentrated hydrochloric acid into a 2-liter reaction vessel fitted with a thermometer, an agitator and a reflux condenser. The reaction mixture was then heated to a temperature between 80° and 85° C. and maintained at that temperature with agitation for a period of 6 hours. At the end of this period, ice and about 500 ml of water were added to the reaction mixture to cool it. After the material had reached room temperature, about 500 ml of methylene chloride was added to the mixture to extract soluble organic constit-

uents and the materials were transferred to a separatory funnel.

The heavier methylene chloride layer was separated from the lighter materials, washed with water, washed twice with a dilute potassium carbonate solution and then again washed with water. The resultant solution was then dried by adding magnesium sulfate and filtered. Following the filtration step, the methylene chloride was removed by distillation. Vacuum distillation of the residue yielded 137 g. of a yellow solid which boiled between 181° C. and 225° C. at a pressure of between 1 and 2 mm of mercury.

Upon recrystallization of this material from ether and hexane, 117 g. of a yellow solid was recovered. Elemental analysis showed a chlorine content of from 9.40 to 9.63% by weight, compared to a theoretical value of 15.64%. The product was then subjected to nuclear magnetic resonance analysis and infrared analysis. Both indicated that ring chloromethylation had occurred and that the product was impure chloromethylphenanthrene.

90 g. of the chloromethylphenanthrene prepared above was placed in a reaction vessel, along with 61.5 g. of crude quinoline. The resulting mixture was then stirred and heated to a temperature of 125° C. A total of 101 g. of isopropanol was weighed out and a portion of this was added to the reaction mixture to permit temperature maintenance of the reaction mixture by refluxing of the isopropanol portion. After the mixture had been held at 125° C. temperature for about 3 hours, the material was cooled to room temperature and the remainder of the isopropanol was added. This resulted in a 60% isopropanol solution of N-(phenanthrylmethyl) quinolinium chloride.

#### EXAMPLE 3

A 250 ml reaction flask was equipped with a thermometer, a stirring device, a reflux condenser and a gas inlet tube. This reactor was charged with 104.14 g. of a polystyrene having a molecular weight of about 250. The material used is marketed by Pennsylvania Industrial Chemicals, Inc. under the tradename of "Piccolastic AL". To this were added 30.3 g. of paraformaldehyde and 30.0 g. of anhydrous zinc chloride.

The resulting mixture was stirred vigorously and then heated to a temperature of 60° C. A stream of hydrogen chloride gas was added through the gas inlet tube at a rate determined by the exothermic heat of reaction. The total reaction time was about 45 minutes. The reaction mixture was then cooled and about 500 ml. of water were added.

Following this, the product was extracted with about 200 ml. of ether and the ether extract was washed twice with 500 ml. of water, once with 500 ml. of saturated sodium bicarbonate, and two more times with water. This extract was then dried twice over magnesium sulfate.

The dried extract was placed in a still and heated to a maximum hot temperature of 128° C. The highest vapor temperature obtained was 38° C. The residue obtained was 94.5 g. of crude chloromethylated low molecular weight polystyrene. Elemental analysis showed the presence of 10.49 to 10.71% chlorine and nuclear magnetic resonance and infrared analysis confirmed that the ring structure had been chloromethylated.

The chloromethylated polystyrene prepared as described above was reacted with quinoline to form the

quaternary derivatives by charging 84.5 g. of the chloromethylated polystyrene, 87 g. of crude quinoline and 85.5 g. of formamide into a reaction vessel, heating the reaction mixture to a temperature of 125° C., and maintaining it at that temperature for a period of 2.5 hours. Following this, the reaction product was cooled slowly to room temperature and 86.0 g. of additional formamide was added. This gave a formamide solution containing approximately 60% by weight of the quaternary derivatives of quinoline and chloromethylated polystyrene.

#### EXAMPLE 4

A heavy aromatic petroleum fraction having a flash point of about 150° F. and consisting primarily of C<sub>9</sub> to C<sub>12</sub> aromatic hydrocarbons was charged into a reaction vessel equipped with a thermometer, a stirrer, a gas inlet tube and a condenser. To 592 g. of this aromatic material was added 134 g. of paraformaldehyde and 120 g. of anhydrous zinc chloride. The reactor contents were brought up to a temperature of 60° C. with vigorous stirring. Dry hydrogen chloride gas was added through the gas inlet tube until a total of 151 g. had been added. About 147 g. of this gas was absorbed in the reaction medium. The total reaction time at 60° C. was 2 hours. The reaction mixture was then cooled and about 500 ml. of water were added. Following this, the product was extracted with about 200 ml. of ether. After separation of the extract, the extracted material was washed twice with water, once with 500 ml. of saturated sodium bicarbonate solution and two more times with water. Following this the extract was dried twice over magnesium sulfate and then the solvent was removed by distillation.

The resultant product (yield=540 g.) contained 12.76 to 12.88% chlorine. Nuclear magnetic resonance and infrared spectroscopy indicated that the product was chloromethylated.

This product (123 g.) was allowed to react with 100 g. of crude quinoline at a temperature of 125° C. in the presence of isopropanol, in a reaction procedure similar to that described above. The quaternarization reaction was carried out over a 5-hour period. Additional isopropanol was added to give a 60 weight percent solution of the mixed quaternary derivative and isopropanol.

#### EXAMPLE 5

A lower boiling aromatic fraction similar to that used in Example 4 above but having a flash point of about 100° F. and containing primarily C<sub>9</sub> aromatics was chloromethylated in a manner similar to that described in Example 4. A 500 g. sample of the aromatic fraction was used and a yield of 574 g. of product was obtained. Nuclear magnetic resonance and infrared spectroscopy confirmed the introduction of the chloromethyl group into the ring structure. Elemental analysis showed a chlorine content of from 16.25 to 16.31%.

A sample of 123 g. of this reaction product was allowed to react with 100 g. of crude quinoline at 125° C. for a period of about 4 hours in the presence of isopropanol. The final aromatic quaternary compound was made up as a 60% solution in isopropanol.

#### EXAMPLE 6

To test the quaternary aromatic compounds prepared as described above, a series of corrosion tests were carried out with 28% hydrochloric acid solutions

on steel coupons. These tests were conducted by first preparing a stock (standard) corrosion inhibitor solution containing 7.5% by weight of a crude grade of 1-hexyne-3-ol, 1.0 weight percent of isoctylphenol polyethyleneoxyethanol containing from 9 to 10 mols of ethylene oxide per mol of isoctylphenol, and 91.5 weight percent of formamide. This inhibitor solution was added in a concentration of 5% by volume to each of a series of bottles containing 100 ml. of 28% hydrochloric acid solution. Samples of the polycyclic quaternary products prepared in Examples 1 through 5 and, for purposes of comparison, samples of N-benzyl-quinolinium chloride (60% in isopropanol) and N-octylquinolinium bromide (60% in isopropanol) were added to separate bottles in concentrations of 0.75 and 1.5% by volume, based on the acid solution. The resulting corrosion inhibition was the total effect of the stock corrosion inhibitor and the quaternary compounds.

The steel coupons used in the tests were cut from new oil field tubing. The coupons were washed with xylene and dried, tumbled in an abrasive compound to remove mill scale, and then scrubbed and acidized briefly in dilute hydrochloric acid. Following this treatment, each coupon was washed and dried and then stored in a dessicator. The coupons measured 1.38 in. long by 1.38 in. wide and retained the curvature of the pipe. Each coupon was weighed before it was used so that the amount of corrosion could be determined. The steel from which the coupons were cut was ASTM P-105 steel.

The tests were carried out by placing a weighed coupon in each of the prepared bottles containing 28% hydrochloric acid and an inhibitor composition. These bottles were then placed in an autoclave and subjected to a temperature of 325° F. and a pressure of 1000 psig for a period of 2 hours. At the end of this period, the samples were removed from the bottles, washed and dried, and then weighed to determine the weight loss. The corrosion rate in pounds per square foot of metal was calculated. The results obtained are set forth in Table I below.

TABLE I

| Corrosion Tests of Quaternaries |                                                                      |                      |                                   |
|---------------------------------|----------------------------------------------------------------------|----------------------|-----------------------------------|
| Test No.                        | Quaternary Compound                                                  | Concentration Vol. % | Corrosion Rate Lb/ft <sup>2</sup> |
| 1                               | Quinoline- $\alpha$ -chloromethyl-naphthalene                        | 0.75                 | 0.0183                            |
| 2                               | Quinoline- $\alpha$ -chloromethyl-naphthalene                        | 1.50                 | 0.0543                            |
| 3                               | Quinoline-chloromethylated polystyrene                               | 0.75                 | 0.140                             |
| 4                               | Quinoline-chloromethylated polystyrene                               | 1.50                 | 0.167                             |
| 5                               | Quinoline-chloromethylated C <sub>9</sub> -C <sub>12</sub> aromatics | 0.75                 | 0.240                             |
| 6                               | Quinoline-chloromethylated C <sub>9</sub> -C <sub>12</sub> aromatics | 1.50                 | 0.260                             |
| 7                               | Quinoline-chloromethylated C <sub>9</sub> aromatics                  | 0.75                 | 0.129                             |
| 8                               | Quinoline-chloromethylated C <sub>9</sub> aromatics                  | 1.50                 | 0.187                             |
| 9                               | Quinoline-Benzyl Chloride                                            | 0.75                 | 0.538                             |
| 10                              | Quinoline-Benzyl Chloride                                            | 1.50                 | 0.359                             |
| 11                              | Quinoline-Octyl Bromide                                              | 0.75                 | 0.413                             |

Note

All test solutions contained 5% by volume of a stock inhibitor consisting of 7.5 wt. % 1-hexyne-3-ol, 91.5 wt. % formamide and 1.0 wt. % of "TRITON X-100" (isoctylphenol polyethyleneoxyethanol).

It will be noted from the above table that the corrosion rates with the samples containing the quaternary compound prepared from quinoline and polycyclic

aromatic materials were less than one-half those obtained with the quinoline-benzyl chloride and quinoline-octyl bromide compounds. The corrosion rates with the quinoline- $\alpha$ -chloromethyl naphthalene quaternary compounds were particularly low.

Earlier work by applicants has shown that the quinoline-benzyl chloride and quinoline-octyl bromide quaternaries are somewhat more effective than materials prepared from other aliphatic and single ring aromatic precursors.

These data thus demonstrate that, in the presence of an acetylenic alcohol, a surface active agent and a formic acid derivative, the specially selected quaternary compounds which have been prepared from quinoline and polycyclic aromatics are surprisingly much more effective than the corresponding materials prepared from aliphatic and single ring aromatic precursors.

#### EXAMPLE 7

Another series of tests similar to that described in Example 6 was carried out using the quinoline-C<sub>9</sub> to C<sub>12</sub> aromatic quaternary of Example 4, the quinoline-C<sub>9</sub> aromatic quaternary of Example 5 and, for purposes of comparison, the quinoline-benzyl chloride quaternary referred to in Example 6. These tests were carried out by preparing 100 ml. samples of 15% hydrochloric acid containing 5% by volume of the base inhibitor described in Example 6 and adding a coupon of P-105 steel to each bottle. The bottles were placed in an autoclave and subjected to a temperature of 350° F. at a pressure of 4000 psig for 2 hours. At the end of this time, the coupons were removed from the bottles, washed and dried, and weighed to permit calculation of the corrosion rate. The results are set forth in Table II below.

TABLE II

| Corrosion Tests in 15% HCl |                                                                      |                              |                                         |
|----------------------------|----------------------------------------------------------------------|------------------------------|-----------------------------------------|
| Test No.                   | Quaternary Compound                                                  | Concen-<br>tration<br>Vol. % | Corrosion<br>Rate<br>Lb/ft <sup>2</sup> |
| 1                          | Quinoline-chloromethylated C <sub>9</sub> -C <sub>12</sub> Aromatics | 0.75                         | 0.0425                                  |
| 2                          | Quinoline-chloromethylated C <sub>9</sub> -Aromatics                 | 1.50                         | 0.0325                                  |
| 3                          | Quinoline-chloromethylated C <sub>9</sub> Aromatics                  | 0.75                         | 0.0439                                  |
| 4                          | Quinoline-chloromethylated C <sub>9</sub> Aromatics                  | 1.50                         | 0.0353                                  |
| 5                          | Quinoline-benzyl Chloride                                            | 0.75                         | 0.0729                                  |
| 6                          | Quinoline-benzyl Chloride                                            | 1.50                         | 0.0706                                  |

Note  
All test solutions contained 5% by volume of a stock inhibitor consisting of 7.5 wt. % 1-hexyn-3-ol, 91.5 wt. % formamide and 1.0 wt. % of "TRITON X-100".

As can be seen from the above Table II, corrosion rates with the samples containing the quaternary compounds prepared from quinoline and the polycyclic aromatic materials were only a little more than about half those obtained with the quinoline-benzyl chloride quaternary. The rates with the quaternary prepared from the C<sub>9</sub> aromatics and that prepared from the C<sub>9</sub>-C<sub>12</sub> aromatics were about the same. All of the rates were considerably lower than those in the earlier tests because of the less concentrated hydrochloric acid and higher pressure used. The corrosion rate normally decreases with increasing pressure when formic acid derivatives are employed in these tests, but this is offset to a large extent in well-treating operations by the higher

temperatures which are generally encountered in deep, high pressure wells.

#### EXAMPLE 8

5 A corrosion inhibitor was formulated by blending formamide, 1-hexyn-3-ol, octylphenolpolyethyleneoxyethanol containing from 8 to 10 mols of ethylene oxide per molecule, the quinoline- $\alpha$ -chloromethyl naphthalene quaternary prepared as described in Example 1, and a fluorinated cationic surfactant to produce a blend having the following composition:

|    | Constituent                                              | Percentage  |
|----|----------------------------------------------------------|-------------|
| 15 | Formamide                                                | 50.5 wt. %  |
|    | 1-hexyn-3-ol                                             | 10.0 wt. %  |
|    | Octylphenolpolyethyleneoxyethanol                        | 2.5 wt. %   |
|    | Fluorinated surfactant                                   | 0.2 wt. %   |
| 20 | Quinoline- $\alpha$ -chloromethyl-naphthalene quaternary | 38.55 wt. % |

25 Samples of the above composition were added to separate bottles containing 100 ml. of 28% hydrochloric acid solution and coupons of P-105, N 80 and C 75 steel. Inhibitor concentrations of 1%, 2% and 3% by volume were used. For purposes of comparison, similar test samples containing two of the best commercially available high temperature corrosion inhibitors were also tested. These test bottles were placed in an autoclave and maintained at 275° F. and 100 psig for a period of 6 hours. The coupons were then removed from the bottles, washed and dried, and weighed for determination of the corrosion rate. The results of these tests are shown in Table III below.

TABLE III

| Tests of Commercial Inhibitors and the Inhibitor of the Invention |            |                              |                |                                       |
|-------------------------------------------------------------------|------------|------------------------------|----------------|---------------------------------------|
| 40                                                                | Inhibitor* | Concen-<br>tration<br>Vol. % | Coupon<br>Type | Corrosion Rate,<br>Lb/ft <sup>2</sup> |
| 45                                                                | A          | 3                            | P 105          | 0.739                                 |
|                                                                   | A          | 3                            | N 80           | 0.664                                 |
|                                                                   | A          | 3                            | C 75           | 0.238                                 |
|                                                                   | B          | 3                            | C 75           | 0.0921                                |
|                                                                   | C          | 1                            | P 105          | 0.276                                 |
|                                                                   | C          | 1                            | N 80           | 0.217                                 |
|                                                                   | C          | 1                            | C 75           | 0.122                                 |
|                                                                   | C          | 2                            | P 105          | 0.0202                                |
| 50                                                                | C          | 2                            | N 80           | 0.0274                                |
|                                                                   | C          | 2                            | C 75           | 0.0264                                |
|                                                                   | C          | 3                            | P 105          | 0.0255                                |
|                                                                   | C          | 3                            | N 80           | 0.0301                                |
|                                                                   | C          | 3                            | C 75           | 0.0464                                |

\*Inhibitor A - Commercially marketed inhibitor.

Inhibitor B - Another commercially marketed inhibitor.

Inhibitor C - Inhibitor composition of the invention.

55 It can be seen from the table that the inhibitor of the invention was more effective at a concentration of 1% than commercial inhibitor A was at a concentration of 3% and about twice as effective as commercial inhibitor B at a concentration of 3%. The data also demonstrate that the improved inhibitor composition of the invention can be used for the protection of various steels and, unlike commercial inhibitor A, does not show wide variations in the level of protection afforded with the three steels tested.

60 Under the particular test conditions employed, the inhibitor composition was most effective at a concentration between 1 and 2 volume percent, based upon the acid. The above data demonstrate that the inhibi-

tors of the invention are surprisingly more effective than the commercial inhibitors available heretofore.

### EXAMPLE 9

Further corrosion tests were carried out using the inhibitor composition of Example 8 and a base inhibitor composition prepared by blending formamide, the fluorinated cationic surfactant of Example 8, a crude 1-hexyn-3-ol and the N-( $\alpha$ -naphthylmethyl)quinucluomchloride of Example 1.

To separate samples of this base inhibitor composition were added three different polyethoxylated primary amines in various concentrations. Coupons of N 80 steel were placed in each of a series of test bottles containing 100 ml. of 15% hydrochloric acid containing the base inhibitor composition in a concentration of 2 volume percent.

The test bottles were placed in an autoclave and held at a temperature of 300° F. and a pressure of 4000 psig for a period of 6 hours. Each sample, after being washed and dried, was weighed to permit determination of the corrosion rate. Table IV below sets forth the results obtained.

TABLE IV

## Use of Polyethoxylated Amines in Inhibitors

| Inhibitor* | Polyethoxylated Amine                                                                                                                                                                       | Surfactant Concentration, Vol. % Based on Acid | Corrosion Rate lb/ft <sup>2</sup> |
|------------|---------------------------------------------------------------------------------------------------------------------------------------------------------------------------------------------|------------------------------------------------|-----------------------------------|
| 1          | —                                                                                                                                                                                           | —                                              | 0.149                             |
| 2          | $\text{C}_{12}\text{H}_{25}-\overset{\text{CH}_2\text{CH}_2\text{OH}}{\underset{\text{CH}_2\text{CH}_2\text{OH}}{\text{N}}}-\text{CH}_2\text{CH}_2\text{OH}$                                | 0.025                                          | 0.0552                            |
| 2          | "                                                                                                                                                                                           | 0.05                                           | 0.0845                            |
| 2          | "                                                                                                                                                                                           | 0.10                                           | 0.0371                            |
| 2          | $\text{C}_{18}\text{H}_{37}-\overset{(\text{CH}_2\text{CH}_2\text{O})_3\text{H}}{\underset{(\text{CH}_2\text{CH}_2\text{O})_2\text{H}}{\text{N}}}-\text{CH}_2\text{CH}_2\text{O}_3\text{H}$ | 0.025                                          | 0.0274                            |
| 2          | "                                                                                                                                                                                           | 0.05                                           | 0.0275                            |
| 2          | "                                                                                                                                                                                           | 0.10                                           | 0.0453                            |
| 2          | $\text{C}_{18}\text{H}_{37}-\overset{(\text{CH}_2\text{CH}_2\text{O})_8\text{H}}{\underset{(\text{CH}_2\text{CH}_2\text{O})_7\text{H}}{\text{N}}}-\text{CH}_2\text{CH}_2\text{O}_8\text{H}$ | 0.025                                          | 0.360                             |
| 2          | "                                                                                                                                                                                           | 0.05                                           | 0.0558                            |
| 2          | "                                                                                                                                                                                           | 0.10                                           | 0.0442                            |
| 2          | $\text{C}_{12}\text{H}_{25}-\overset{\text{CH}_2\text{CH}_2\text{OH}}{\underset{\text{CH}_2\text{CH}_2\text{OH}}{\text{N}}}-\text{CH}_2\text{CH}_2\text{OH}$                                | 0.025                                          | 0.0575                            |
| 2          | "                                                                                                                                                                                           | 0.05                                           | 0.0296                            |
| 2          | "                                                                                                                                                                                           | 0.10                                           | 0.0368                            |

\*1 - Inhibitor of Example 8 containing 50.5% formamide, 0.2% perfluoroalkyl-ylimidazoline, 1.25% polyethoxylated octyl phenol, 10.0% hexyne-1-ol-3, and 38.55% N-(anaphthylmethyl) quinolinium chloride.

\*2 - Inhibitor base containing 50.63% formamide, 0.2% perfluoroalkylimidazoline, 10.13% hexyne-1-ol-3, and 39.04% N-( $\alpha$ -naphthylmethyl)quinolinium chloride.

It can be seen from the data of Table IV that inclusion of the polyethoxylated amines in the inhibitor base as a surfactant instead of the polyethoxylated octyl phenol resulted in a considerably higher level of protection for the N 80 steel coupons used in the test than was obtained with the inhibitor composition of Example 8. The  $C_{12}$  alkyl polyethoxylated amine was particu-

larly effective. As a result of this, it is preferred to employ the polyethoxylated amines as the primary surface active agents in the inhibitor compositions of the invention.

### EXAMPLE 10

Still another series of tests was carried out with the inhibitor blend composition of Example 8 and a composition prepared by blending 50 weight percent formamide, 0.2 weight percent of the previously described fluorinated surfactant, 10.0 weight percent of 1-hexyn-10-ol, 28.55 weight percent of the N-( $\alpha$ -naphthylmethyl)quinolinium chloride of Example 1 and 1.25 weight percent of a polyethoxylated C<sub>18</sub> alkyl primary amine containing a total of 5 ethylene oxide groups per molecule. Samples of these two inhibitor blends were 15 added to bottles containing 100 ml. of 15% HCl in an inhibitor concentration of 2%. Coupons of P 105 and N 20 80 steel were placed in separate bottles containing the inhibited acid and these bottles were then placed in the 25 autoclave and held at 300° F. and 4000 psig for 6 hours. The coupons were removed at the end of this period, washed and dried, and weighed for determination of the corrosion rate. Table V below sets forth the results.

TABLE V

| Corrosion Inhibitor Tests |        |                                       |
|---------------------------|--------|---------------------------------------|
| Inhibitor*                | Coupon | Corrosion Rate,<br>Lb/ft <sup>2</sup> |
| 1                         | P 105  | 0.0292                                |
| 1                         | N 80   | 0.178                                 |
| 2                         | P 105  | 0.0589                                |
| 2                         | N 80   | 0.0376                                |

\*1 - Inhibitor of Example 8 containing 50.0% formamide, 0.2% perfluoroalkylimidazoline, 1.25% polyethoxylated octyl phenol, 10.0% 1-hexyn-3-ol, and 38.55% NaCl, and 1.0% diisopropylcarbonyldiimidazole.

38.55% N-(*α*-naphthylmethyl)quinolinium chloride.  
 \*2 - Inhibitor containing 50.0% formamide, 0.2% perfluoroalkylimidazoline, 10.0% hexyne-1-ol-3, 38.55% N-(*α*-naphthylmethyl)quinolinium chloride, and 1.25% C<sub>12</sub> alkyl polyethoxylated amine containing 5 ethylene oxide groups.

Although both of the inhibitors used in the tests reported above were reasonably effective under the test conditions employed, it is clear that Inhibitor 2 was more effective than the material of Example 8. This composition is therefore a particularly preferred one for the purposes of the invention.

**EXAMPLE 11**

60 The following experimental result demonstrates the importance of utilizing a polynuclear heterocyclic amine and a polynuclear quaternizing agent in formulating the corrosion inhibiting compositions of the present invention. Adducts of various heterocyclic amines were prepared with  $\alpha$ -chloromethylnaphthalene according to the following equation and following the general procedures set forth in detail in the previous examples.



The adducts were prepared either as a 60% solution in isopropanol if they were suitably soluble or isolated as a solid if they precipitated.

The results of two tests are summarized below in Table VI.

TABLE VI

| Test Conditions                                               |                                        | Test Results Summary<br>Reported in<br>Corrosion (lb/ft <sup>2</sup> ) |        |       |
|---------------------------------------------------------------|----------------------------------------|------------------------------------------------------------------------|--------|-------|
| Heterocyclic Adduct                                           | Comment                                | Test 1                                                                 | Test 2 | Avg.  |
| N-(naphthylmethyl) quinolinium chloride                       | Prepared from crude grade of quinoline | 0.113                                                                  | 0.0965 | 0.105 |
| N-(naphthylmethyl) quinolinium chloride                       | Prepared from reagent grade quinoline  | 0.316                                                                  | 0.165  | 0.240 |
| N-(naphthylmethyl) (5, 6 benzoquinolinium) chloride           |                                        | 0.367                                                                  | 0.320  | 0.344 |
| N-(naphthylmethyl) acridinium chloride                        |                                        | 0.0513                                                                 | 0.074  | 0.063 |
| N-(naphthylmethyl) phenanthridinium chloride                  |                                        | 0.117                                                                  | 0.103  | 0.110 |
| N-(naphthylmethyl) pyridinium chloride                        |                                        | 0.547                                                                  | 0.590  | 0.568 |
| Blank No.1 (No quaternary compound)                           |                                        | 1.04                                                                   | 0.960  | 1.00  |
| Blank No.2 (No stock inhibitor and<br>No quaternary compound) |                                        | 1.08                                                                   | 1.11   | 1.10  |

The above tests demonstrate the remarkable dependence on the type of heterocyclic amine, as well as the necessity of a quaternary adduct in these types of systems. The unusual high performance of the acridine and phenanthridine adduct is unexpected. The poor performance of the pyridine adduct is also noteworthy since it strongly supports the criticality aspects of the invention.

## EXAMPLE 12

The following is a hypothetical example to illustrate the use of the Supplemental Surfactant.

A. To the blend of Example 8 is added 10 wt. % of BR1J-35.

B. To the blend of Example 9 containing the C<sub>12</sub> alkyl polyethoxylated amine is added 10 wt. % of BR1J-35.

The fluorocarbon surfactant used in the examples is cationic and was obtained from Minnesota Mining and Manufacturing Company under the trademark "FC-134". This is a typical fluorocarbon surfactant. There

50  
55



where R is an aliphatic, alicyclic or aromatic residue containing from 1 to about 12 carbon atoms and may include one or more functional groups such as halogen atoms, carbonyl, carboxyl, carbamyl, amino, formyl or nitroso radicals or other functional groups without impaired performance.

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
7710  
7711  
7712  
7713  
7714  
7715  
7716  
7717  
7718  
7719  
7720  
7721  
7722  
7723  
7724  
7725  
7726  
7727  
7728  
7729  
7730  
7731  
7732  
7733  
7734  
7735  
7736  
7737  
7738  
7739  
7740  
7741  
7742  
7743  
7744  
7745  
7746  
7747  
7748  
7749  
7750  
7751  
7752  
7753  
7754  
7755  
7756  
7757  
7758  
7759  
7760  
7761  
7762  
7763  
7764  
7765  
7766  
7767  
7768  
7769  
7770  
7771  
7772  
7773  
7774  
7775  
7776  
7777  
7778  
7779  
77710  
77711  
77712  
77713  
77714  
77715  
77716  
77717  
77718  
77719  
77720  
77721  
77722  
77723  
77724  
77725  
77726  
77727  
77728  
77729  
77730  
77731  
77732  
77733  
77734  
77735  
77736  
77737  
77738  
77739  
77740  
77741  
77742  
77743  
77744  
77745  
77746  
77747  
77748  
77749  
77750  
77751  
77752  
77753  
77754  
77755  
77756  
77757  
77758  
77759  
77760  
77761  
77762  
77763  
77764  
77765  
77766  
77767  
77768  
77769  
77770  
77771  
77772  
77773  
77774  
77775  
77776  
77777  
77778  
77779  
77780  
77781  
77782  
77783  
77784  
77785  
77786  
77787  
77788  
77789  
77790  
77791  
77792  
77793  
77794  
77795  
77796  
77797  
77798  
77799  
777100  
777101  
777102  
777103  
777104  
777105  
777106  
777107  
777108  
777109  
777110  
777111  
777112  
777113  
777114  
777115  
777116  
777117  
777118  
777119  
777120  
777121  
777122  
777123  
777124  
777125  
777126  
777127  
777128  
777129  
777130  
777131  
777132  
777133  
777134  
777135  
777136  
777137  
777138  
777139  
777140  
777141  
777142  
777143  
777144  
777145  
777146  
777147  
777148  
777149  
777150  
777151  
777152  
777153  
777154  
777155  
777156  
777157  
777158  
777159  
777160  
777161  
777162  
777163  
777164  
777165  
777166  
777167  
777168  
777169  
777170  
777171  
777172  
777173  
777174  
777175  
777176  
777177  
777178  
777179  
777180  
777181  
777182  
777183  
777184  
777185  
777186  
777187  
777188  
777189  
777190  
777191  
777192  
777193  
777194  
777195  
777196  
777197  
777198  
777199  
777200  
777201  
777202  
777203  
777204  
777205  
777206  
777207  
777208  
777209  
777210  
777211  
777212  
777213  
777214  
777215  
777216  
777217  
777218  
777219  
777220  
777221  
777222  
777223  
777224  
777225  
777226  
777227  
777228  
777229  
777230  
777231  
777232  
777233  
777234  
777235  
777236  
777237  
777238  
777239  
777240  
777241  
777242  
777243  
777244  
777245  
777246  
777247  
777248  
777249  
777250  
777251  
777252  
777253  
777254  
777255  
777256  
777257  
777258  
777259  
777260  
777261  
777262  
777263  
777264  
777265  
777266  
777267  
777268  
777269  
777270  
777271  
777272  
777273  
777274  
777275  
777276  
777277  
777278  
777279  
777280  
777281  
777282  
777283  
777284  
777285  
777286  
777287  
777288  
777289  
777290  
777291  
777292  
777293  
777294  
777295  
777296  
777297  
777298  
777299  
777300  
777301  
777302  
777303  
777304  
777305  
777306  
777307  
777308  
777309  
777310  
777311  
777312  
777313  
777314  
777315  
777316  
777317  
777318  
777319  
777320  
777321  
777322  
777323  
777324  
777325  
777326  
777327  
777328  
777329  
777330  
777331  
777332  
777333  
777334  
777335  
777336  
777337  
777338  
777339  
777340  
777341  
777342  
777343  
777344  
777345  
777346  
777347  
777348  
777349  
777350  
777351  
777352  
777353  
777354  
777355  
777356  
777357  
777358  
777359  
777360  
777361  
777362  
777363  
777364  
777365  
777366  
777367  
777368  
777369  
777370  
777371  
777372  
777373  
777374  
777375  
777376  
777377  
777378  
777379  
777380  
777381  
777382  
777383  
777384  
777385  
777386  
777387  
777388  
777389  
777390  
777391  
777392  
777393  
777394  
777395  
777396  
777397  
777398  
777399  
777400  
777401  
777402  
777403  
777404  
777405  
777406  
777407  
777408  
777409  
777410  
777411  
777412  
777413  
777414  
777415  
777416  
777417  
777418  
777419  
777420  
777421  
777422  
777423  
777424  
777425  
777426  
777427  
777428  
777429  
777430  
777431  
777432  
777433  
777434  
777435  
777436  
777437  
777438  
777439  
777440  
777441  
777442  
777443  
777444  
777445  
777446  
777447  
777448  
777449  
777450  
777451  
777452  
777453  
777454  
777455  
777456  
777457  
777458  
777459  
777460  
777461  
777462  
777463  
777464  
777465  
777466  
777467  
777468  
777469  
777470  
777471  
777472  
777473  
777474  
777475  
777476  
777477  
777478  
777479  
777480  
777481  
777482  
777483  
777484  
777485  
777486  
777487  
777488  
777489  
777490  
777491  
777492  
777493  
777494  
777495  
777496  
777497  
777498  
777499  
777500  
777501  
777502  
777503  
777504  
777505  
777506  
777507  
777508  
777509  
777510  
777511  
777512  
777513  
777514  
777515  
777516  
777517  
777518  
777519  
777520  
777521  
777522  
777523  
777524  
777525  
777526  
777527  
777528  
777529  
777530  
777531  
777532  
777533  
777534  
777535  
777536  
777537  
777538  
777539  
777540  
777541  
777542  
777543  
777544  
777545  
777546  
777547  
777548  
777549  
777550  
777551  
777552  
777553  
777554  
777555  
777556  
777557  
777558  
777559  
777560  
777561  
777562  
777563  
777564  
777565  
777566  
777567  
777568  
777569  
777570  
777571  
777572  
777573  
777574  
777575  
777576  
777577  
777578  
777579  
777580  
777581  
777582  
777583  
777584  
777585  
777586  
777587  
777588  
777589  
777590  
777591  
777592  
777593  
777594  
777595  
777596  
777597  
777598  
777599  
777600  
777601  
777602  
777603  
777604  
777605  
777606  
777607  
777608  
777609  
777610  
777611  
777612  
777613  
777614  
777615  
777616  
777617  
777618  
777619  
777620  
777621  
777622  
777623  
777624  
777625  
777626  
777627  
777628  
777629  
777630  
777631  
777632  
777633  
777634  
777635  
777636  
777637  
777638  
777639  
777640  
777641  
777642  
777643  
777644  
777645  
777646  
777647  
777648  
777649  
777650  
777651  
777652  
777653  
777654  
777655  
777656  
777657  
777658  
777659  
777660  
777661  
777662  
777663  
777664  
777665  
777666  
777667  
777668  
777669  
777670  
777671  
777672  
777673  
777674  
777675  
777676  
777677  
777678  
777679  
777680  
777681  
777682  
777683  
777684  
777685  
777686  
777687  
777688  
777689  
777690  
777691  
777692  
777693  
777694  
777695  
777696  
777697  
777698  
777699  
777700

1. from about 25 to about 60 weight percent of a quaternary compound of (i) a heterocyclic nitrogen base selected from the group consisting of quinoline, acridine and phenanthridine and (ii) a halomethylated polycyclic aromatic compound selected from the group consisting of halomethylated indane, indene, naphthalene, anthracene, phenanthrene, acenaphthene, fluorene, xanthene, chrysene and pyrene, halomethylated petroleum fractions containing  $C_9$  to  $C_{12}$  aromatic hydrocarbons, and halomethylated polystyrenes having molecular weights ranging from about 100 to about 5,000;
2. from about 5 to about 30 weight percent of an aliphatic acetylenic alcohol having the structural formula of



wherein  $R_1$  is selected from the group consisting of hydrogen and a methyl group and  $R_2$  is selected from the group consisting of hydrogen and alkyl groups containing from 1 to about 7 carbon atoms;

3. from about 0.01 to about 15 weight percent of a water-soluble surface active agent selected from the group consisting of polyethoxylated octyl phenol and polyethoxylated amines having the structural formula of



35

wherein R is a  $C_5$  to  $C_{50}$  alkyl group, and m and n are numbers ranging from 1 to about 20; and

4. from about 30 to about 75 weight percent of a formic acid derivative having the formula of



40

wherein Z is selected from the group consisting of an alkoxy group containing from 1 to about 4 carbon atoms, an amino radical, and an alkyl-substituted amino group containing from 1 to about 4 carbon atoms.

2. The composition of claim 1 wherein said quaternary compound is N-( $\alpha$ -naphthylmethyl) quinolinium chloride.

3. The composition of claim 1 wherein said surface active agent is polyethoxylated octyl phenol.

4. The composition of claim 2 wherein said surface active agent is polyethoxylated octyl phenol.

5. The composition of claim 1 wherein said acetylenic alcohol is 1-hexyn-3-ol.

6. The composition of claim 1 wherein said formic acid derivative is formamide.

7. The composition of claim 1 wherein said surface active agent is a polyethoxylated amine of the general formula



60

wherein R is a  $C_5$  to  $C_{50}$  alkyl group and n is a number of between 1 to 20.

8. The composition of claim 1 which contains from 6 to 14 weight percent of a supplementary surfactant comprising the reaction product of lauryl alcohol with about 20 to 23 moles of ethylene oxide.

9. The composition of claim 1 wherein said quaternary compound is N-( $\alpha$ -naphthylmethyl) quinolinium chloride, said acetylenic alcohol is hexyne-1-ol-3 and said formic acid derivative is formamide.

10. The composition of claim 9 wherein said surface active agent is polyethoxylated octyl phenol.

11. The composition of claim 1 wherein said heterocyclic nitrogen base is acridine.

12. The composition of claim 1 wherein said heterocyclic nitrogen base is phenanthridine.

13. The composition of claim 1 wherein said surface active agent is selected from the group consisting of polyethoxylated amines having the structural formula of:



wherein R is a  $C_{12}$  to  $C_{18}$  alkyl group, and m and n are numbers ranging from 1 to about 8.

14. A corrosion inhibitor composition comprising:

1. from about 25 to about 60 weight percent of a quaternary compound of (i) a heterocyclic nitrogen base selected from the group consisting of acridine and phenanthridine and (ii) a halomethylated polycyclic aromatic compound selected from the group consisting of halomethylated indane, indene, naphthalene, anthracene, phenanthrene, acenaphthene, fluorene, xanthene, chrysene and pyrene, halomethylated petroleum fractions containing  $C_9$  to  $C_{12}$  aromatic hydrocarbons, and halomethylated polystyrenes having molecular weights ranging from about 100 to about 5,000;

2. from about 5 to about 30 weight percent of an aliphatic acetylenic alcohol having the structural formula of



wherein  $R_1$  is selected from the group consisting of hydrogen and a methyl group, and  $R_2$  is selected from the group consisting of hydrogen and alkyl groups containing from 1 to about 7 carbon atoms;

3. from about 0.01 to about 15 weight percent of a water-soluble surface active agent selected from the group consisting of polyethoxylated amines having the structural formula of



65 where R is a  $C_{12}$  to  $C_{18}$  alkyl group, m and n are numbers ranging from 1 to about 8; and

4. from about 30 to about 75 weight percent of a formic acid derivative having the formula of



wherein Z is selected from the group consisting of an alkoxy group containing from 1 to about 4 carbon atoms, an amino radical and an alkyl-substituted amino group containing from 1 to about 4 carbon atoms.

15. The composition of claim 14 wherein said heterocyclic nitrogen base is acridine.

16. The composition of claim 15 wherein said quaternary compound is N-(naphthylmethyl)-acridinium chloride.

17. The composition of claim 14 wherein said heterocyclic nitrogen base is phenanthridine.

18. The composition of claim 17 wherein said quaternary compound is N-(naphthylmethyl)-phenanthridinium chloride.

19. The composition of claim 14 wherein said surface active agent is a polyethoxylated amine having the structural formula of:



5



10 20. The composition of claim 14 wherein said surface active agent is a polyethoxylated amine having the structural formula of:



15 20. The composition of claim 14 wherein said surface active agent is a polyethoxylated amine having the structural formula of:



\* \* \* \* \*

30

35

40

45

50

55

60

65